

Nov. 3, 1936.

E. J. WARD

2,059,829

SENSITIVE PHOTOGRAPHIC ELEMENT

Filed Nov. 1, 1934

Fig.1.



Fig.2.



Inventor:

Erwin J. Ward,

Newton M. Perrino

By

Attorney

## UNITED STATES PATENT OFFICE

2,059,829

## SENSITIVE PHOTOGRAPHIC ELEMENT

Erwin J. Ward, Rochester, N. Y., assignor, by  
mesne assignments, to Eastman Kodak Com-  
pany, Jersey City, N. J., a corporation of New  
Jersey

Application November 1, 1934, Serial No. 751,007

11 Claims. (Cl. 95—8)

This invention relates to photographic elements including, particularly in the sensitive layer, a material which renders film and especially the emulsion less susceptible to abrasion, both before and after processing, as well as to decrease the coefficient of friction so that photographic material may be moved over a metal or other surface with less wear than would otherwise be the case. I have discovered that if, to any ordinary gelatino 5 silver halide emulsion or to gelatine, there is added a small proportion of wax or wax-like material, this desirable quality is much increased.

The method of preparation and the type of the emulsion is comparatively immaterial as my experiments have indicated that the wax is inert 15 in ordinary emulsions and does not decrease their keeping properties. The types of emulsions and methods of incorporation may be those referred to in the patent Seel, No. 1,757,482, granted May 6, 1930.

In such emulsions or in any other gelatino silver halide emulsion I include a small proportion of wax. While I find carnauba wax particularly efficacious, I contemplate the use of other natural waxes such as beeswax, Montan or 25 Cantol wax, waxes of mineral origin, such as paraffin and synthetic waxes such as the chlorinated naphthalenes and chlorinated diphenyls, and I include all such substances under the term 30 "wax" when used broadly in the claims. All of these compounds have softening or melting points higher than ordinary or room temperatures, i. e., above about 20° C. and are therefore solid at ordinary temperatures.

An ordinary photographic emulsion can be easily scratched or dug with the finger nail, actually removing portions of the emulsion and leaving visible gouges, while with my improved emulsion, it is very difficult, if not impossible to 35 do more than slightly emboss the surface. In ordinary usage therefore, there will not be produced scratches that may be filled with dirt. It is evident that this function of the wax is of importance primarily at or near the surface and 40 the wax may be incorporated only in the outer stratum of emulsion or in an outer stratum of unsensitized gelatine applied to and unitary with the sensitized gelatine layer. These strata may be formed by successive coating operations as is 45 common in photographic manufacture.

A satisfactory method for the introduction of the wax into the photographic emulsion or gelatine layer is to disperse the wax so that particles are of the order of magnitude of those found in 50 silver halide emulsion, i. e. from 1 to 10 microns.

This may be accomplished through the use of various dispersing agents such as triethanolamine oleate. As an example, a carnauba wax dispersion in water with the dispersing agent is added to the gelatine or to the gelatino silver halide 5 emulsion by heating the latter to approximately 40° C. and introducing the wax dispersion with vigorous dispersion at this temperature. The dispersion may be made at any satisfactory concentration, but it has been found that 5% of 10 carnauba wax is quite satisfactory, although I contemplate a wide variation in proportions from .25 to 25 parts by weight of wax to 100 parts of dry 15 gelatine.

Reference is made to the accompanying draw- 15 ing, the two figures of which show on an exaggerated scale sections of film embodying different embodiments of my invention. In Figure 1, 1 indicates any suitable support, preferably 20 of a cellulose ester composition, and 2 indicates the sensitive layer including wax as an ingre- 25 dient.

In Figure 2, the support 1 carries a composite layer, the inner portion 20 of which is sensitive 25 and free from wax and the outer stratum 21 of which is gelatine-wax layer of the type herein described and which may or may not be sensitized. A gelatine layer 22 containing wax may also be applied to the rear of the film. This layer may 30 contain anti-halation dyes and would be formed in the manner described and have the properties mentioned of lessening friction. Other protein layers may be used, such as casein applied hot. This is then not removable in the processing bath.

While I contemplate the use of my invention 35 particularly in motion picture and sound films, it is obvious that it may be useful in any photographic element, such as film packs, X-ray film and the like; and I consider as within my invention all such modifications and equivalents as 40 may be covered by the appended claims.

Having thus described my invention, what I claim as new and desire to be secured by Letters Patent of the United States is:

1. A photographic element including a sup- 45 port and a gelatino silver halide emulsion thereon containing a small proportion of a wax which is solid at ordinary temperatures finely and uniformly dispersed therein.

2. A photographic element including a sup- 50 port and a gelatino silver halide emulsion thereon containing a small proportion of carnauba wax finely and uniformly dispersed therein.

3. A photographic element including a sup- 55 port and a gelatino silver halide emulsion there-

on containing between  $\frac{1}{4}$  of 1% and 25% of a wax which is solid at ordinary temperatures finely and uniformly dispersed therein.

4. A photographic element including a support and a gelatino silver halide emulsion thereon containing between  $\frac{1}{4}$  of 1% and 25% of a natural wax of vegetable origin finely and uniformly dispersed therein.

5. A photographic element including a support and a gelatino silver halide emulsion thereon containing between  $\frac{1}{4}$  of 1% and 25% of carnauba wax finely and uniformly dispersed therein.

6. A photographic element including a support and a unitary gelatine layer on one face thereof, at least the inner stratum of said layer being photographically sensitive and at least the outer stratum thereof including a small proportion of wax which is solid at ordinary temperatures finely and uniformly mixed in the layer.

7. A photographic element including a support and a unitary gelatine layer on one face thereof, at least the inner stratum of said layer containing sensitive silver salts and at least the outer stratum thereof including a small proportion of a natural wax of vegetable origin finely and uniformly dispersed therein.

8. A photographic sensitive element including a support, on one face thereof a unitary gelatine

layer containing a small proportion of wax finely and uniformly dispersed therein in the body of the layer, and on the opposite face thereof a sensitive emulsion layer.

9. A photographic element including a support and a unitary gelatine layer on one face thereof, the inner stratum of said layer containing sensitive silver salts and the outer stratum thereof including a small proportion of a wax which is solid at ordinary temperatures finely and uniformly dispersed in the layer.

10. A photographic motion picture film comprising a support of cellulose ester composition and a unitary gelatine layer on one face thereof, the inner stratum of said layer containing sensitive silver salts and the outer stratum thereof including a small proportion of a wax which is solid at ordinary temperatures finely and uniformly dispersed in the layer.

11. A photographic motion picture film comprising a support of cellulose ester composition and a unitary gelatine layer on one face thereof, the inner stratum of said layer containing sensitive silver salts and the outer stratum thereof including a small proportion of a natural wax of vegetable origin finely and uniformly dispersed therein.

ERWIN J. WARD.